# EUROPEAN PATENT SPECIFICATION

(11) **EP 2 889 059 B1**
(45) Date of publication and mention of the grant of the patent: **23.08.2017**
(21) Application number: 14200445.6
(22) Date of filing: 29.12.2014
(51) Int. Cl.: A63B 37/00, A63B 45/02

(54) **Golf ball and method for producing the same**
Golfball und Verfahren zur Herstellung davon
Balle de golf et son procédé de production

(30) Priority: 27.12.2013 JP 2013273040; 17.01.2014 JP 2014007120
(43) Date of publication of application: 01.07.2015
(73) Proprietor: Dunlop Sports Co., Ltd., Hyogo 651-0072 (JP)
(72) Inventor: Sajima, Takahiro, Kobe-shi, Hyogo 651-0072 (JP); Mimura, Kohei, Kobe-shi, Hyogo 651-0072 (JP)
(74) Representative: Manitz Finsterwald Patentanwälte PartmbB

(56) References cited:
- EP-A1- 2 671 619
- JP-A- 2006 075 210
- US-A1- 2003 096 663
- US-A1- 2007 026 971
- US-A1- 2012 329 367
- US-A1- 2013 303 309
- US-B1- 6 991 565

## Description

### Technical Field

The present invention relates to a golf ball and a method for producing the same.

### Background Art

A golf ball has a large number of dimples on its surface. The dimples disturb airflow around the golf ball during flight and cause turbulent separation. This phenomenon is referred to as "turbulence". Turbulence causes a separation point of air from the golf ball to shift rearward, and thus drag is reduced. Moreover, turbulence promotes the displacement between an upper separation point and a lower separation point due to backspin, and thus lift acting on the golf ball is enhanced. Accordingly, good dimples disturb airflow better, and thus largely extend the flight-distance.

US 2012/0329367 discloses a golf ball with enhanced micro surface roughness on its exterior surface. Its fig. 12 illustrates the ratio of coefficient of lift against coefficient of drag for roughened balls in accordance with examples of its disclosure and smooth control balls at various Reynolds number and/or other launch conditions.

US 2003/0096663 A1 discloses table 3, showing the results of tests with golf balls, where the lift coefficient and a drag coefficient where measured for given spin amounts and Reynolds numbers.

JP 2006-075, 210 discloses a golf ball having a golf ball body and a coating film covering the golf ball body, wherein the coating film contains metal particles.

EP 2 671 619 A1 relates to a golf ball comprising a golf ball body and a paint film formed on the surface of the golf ball body, wherein the paint film has a certain specific storage modulus.

US 2007/0026971 A1 discloses a golf ball having an outer surface including a plurality of dimples forming indicia.

US 2013/0303309 A1 relates to a golf ball having a core, an intermediate layer and a cover, wherein the intermediate layer is cast from polyurethane or polyuria.

### Citation List

### Patent Literature

Patent Literature 1: JP H10-234885A

### Summary of Invention

### Technical Problem

Incidentally, when a golfer hits a golf ball with a middle iron, for example, a large amount of spin is given to the golf ball. As a result, the golf ball is likely to pop up, and the flight-distance sometimes becomes short. Such a problem is not only associated with middle irons. Conventionally, in order to suppress the pop-up, attempts have been made to improve the dimple specifications when designing the dimples. However, this problem has not been solved yet, and the improvement of aerodynamic performance regardless of the design of dimples has been desired. The present invention was achieved in order to solve the foregoing problems, and it is an object thereof to provide a golf ball that can enhance flight performance.

### Solution to Problem

A golf ball according to the present invention includes a spherical core, at least one cover member that covers the core, and a coating layer that covers the cover member configuring an outermost layer, wherein a plurality of dimples are formed in the cover member configuring the outermost layer, and roughness is formed on a surface of the coating layer such that a relationship between a drag coefficient CD1 and a lift coefficient CL1 when a golf ball is hit with a Reynolds number of 1.771×10⁵ and a spin amount of 2280 rpm satisfies CD1×CL1<0.0370.

In the golf ball, it is possible to form roughness on the surface of the coating layer such that a relationship between a drag coefficient CD2 and a lift coefficient CL2 when a golf ball is hit with a Reynolds number of 1.771×10⁵ and a spin amount of 2940 rpm satisfies CD2xCL2<0.0410.

In the golf ball, it is possible to set an arithmetic average roughness Ra of a surface of the coating layer to be 0.5 µm or more.

In the golf ball, it is possible to set a maximum height Rz to be 4.0 µm or more.

In the golf ball, it is possible to set an arithmetic average roughness Ra of a surface of the coating layer to be 0.5 µm or more and a maximum height Rz to be 4.0 µm or more.

The roughness of the coating layer of the golf ball can be formed by various methods, such as a method in which minute particles are sprayed.

In the golf ball, it is possible to set the average particle diameter of the minute particles to be 50 µm or more.

In the golf ball, it is possible to set the thickness of the coating layer to be 5.0 µm or more and 30µm or less.

A method for producing a golf ball according to the present invention includes a step of forming a spherical core, a step of covering the spherical core with at least one cover member and forming a plurality of dimples in the cover member configuring an outermost layer, a step of covering the cover member configuring the outermost layer with a coating layer, and a step of forming roughness on a surface of the coating layer such that a relationship between a drag coefficient CD1 and a lift coefficient CL1 when a golf ball is hit with a Reynolds number of 1.771×10⁵ and a spin amount of 2280 rpm satisfies CD1×CL1<0.0370.

In the method for producing a golf ball, in the step of forming roughness, it is possible to form roughness on the surface of the coating layer such that a relationship between a drag coefficient CD2 and a lift coefficient CL2 when a golf ball is hit with a Reynolds number of 1.771×10⁵ and a spin amount of 2940 rpm satisfies CD2xCL2<0.0410.

In the method for producing a golf ball, it is possible to set an arithmetic average roughness Ra of the roughness formed on the surface of the coating layer to be 0.5 µm or more.

In the method for producing a golf ball, it is possible to set a maximum height Rz to be 4.0 µm or more.

In the method for producing a golf ball, it is possible to set an arithmetic average roughness Ra of the roughness formed on the surface of the coating layer to be 0.5 µm or more and a maximum height Rz to be 4.0 µm or more.

The roughness of the coating layer of the golf ball in the method can be formed by various methods, such as a method in which minute particles are sprayed.

In the method for producing a golf ball, it is possible to set the average particle diameter of the minute particles to be 50 µm or more.

### Advantageous Effects of Invention

With the golf ball and the method for producing the same according to the present invention, it is possible to enhance flight performance.

### Brief Description of Drawings

FIG. 1 is a partially cutaway cross-sectional view illustrating an embodiment of a golf ball of the present invention.
FIG. 2 is a partially enlarged cross-sectional view of FIG. 1.
FIG. 3 is a schematic diagram illustrating forces acting on a golf ball.

### Description of Embodiments

### 1. Golf ball

Hereinafter, an embodiment of a golf ball according to the present invention will be described with reference to the drawings. FIG. 1 is a partially cutaway cross-sectional view of a golf ball according to this embodiment.

As shown in FIG. 1, the golf ball includes a spherical core 1, an intermediate layer 2 that covers the core 1, a cover 3 that covers the intermediate layer 2, and a coating layer 4 that covers the surface of the cover 3.

The diameter of the golf ball is preferably 40 to 45 mm, and more preferably 42.67 mm or more from the viewpoint of meeting the standards of the United States Golf Association (USGA) . From the viewpoint of suppressing air resistance, the diameter is preferably 44 mm or less, and more preferably 42.80 mm or less. Moreover, the mass of the golf ball is preferably 40 g or more and 50 g or less. In particular, from the viewpoint that a large inertia can be provided, the mass is preferably 44 g or more and more preferably 45.00 g or more. From the viewpoint of meeting the standards of the USGA, the mass is preferably 45.93 g or less.

### 1-1. Core

Next, members configuring the golf ball will be described. The core 1 is formed by crosslinking a rubber composition. Examples of the base rubber for the rubber composition include polybutadiene, polyisoprene, styrene-butadiene copolymer, ethylene-propylene-diene copolymer, and natural rubber. Two or more types of rubber may be used in combination. Moreover, from the viewpoint of restitution performance, polybutadiene is preferable, and high-cis polybutadiene is particularly preferable.

The rubber composition of the core 1 includes a co-crosslinking agent. From the viewpoint of restitution performance, preferable co-crosslinking agents are zinc acrylate, magnesium acrylate, zinc methacrylate, and magnesium methacrylate. It is preferable that the rubber composition includes organic peroxide together with the co-crosslinking agent. Examples of the preferable organic peroxide include dicumyl peroxide, 1,1-bis(t-butylperoxy)-3,3,5-trimethylcyclohexane, 2,5-dimethyl-2,5-di(t-butylperoxy)hexane, and di-t-butyl peroxide.

The rubber composition of the core 1 may include additives such as a filler, sulfur, a vulcanization accelerator, a sulfur compound, an antioxidant, a coloring agent, a plasticizer, a dispersant, a carboxylic acid, and a carboxylate. Furthermore, the rubber composition may include synthetic resin powder or crosslinked rubber powder.

The diameter of the core 1 is preferably 30.0 mm or more, and particularly preferably 38.0 mm or more. On the other hand, the diameter of the core 1 is preferably 42.0 mm or less, and particularly preferably 41.5 mm or less. The core 1 may have two or more layers. There is no particular limitation on the shape of the core 1 as long as the core 1 has a spherical shape as a whole, and the core 1 may have ribs on its surface. Moreover, the core 1 may be hollow.

### 1-2. Intermediate layer

Next, the intermediate layer 2 will be described. The intermediate layer 2 is made of a resin composition. An ionomer resin is a preferable base polymer for the resin composition. One example of a preferable ionomer resin is a bipolymer of α-olefin and α,β-unsaturated carboxylic acid that has 3 to 8 carbon atoms. Another example of a preferable ionomer resin is a terpolymer of α-olefin, α,β-unsaturated carboxylic acid that has 3 to 8 carbon atoms and α,β-unsaturated carboxylic acid ester that has 2 to 22 carbon atoms. In the bipolymer and the terpolymer, ethylene and propylene are preferable α-olefins, and acrylic acid and methacrylic acid are preferable α,β-unsaturated carboxylic acids. In the bipolymer and the terpolymer, some of the carboxyl groups are neutralized by metal ions. Examples of metal ions for neutralization include a sodium ion, potassium ion, lithium ion, zinc ion, calcium ion, magnesium ion, aluminum ion, and neodymium ion.

The resin composition of the intermediate layer 2 may include another polymer instead of the ionomer resin. Other examples of polymers include polystyrene, polyamide, polyester, polyolefin, and polyurethane. The resin composition may include two or more types of polymers.

The resin composition of the intermediate layer 2 may include a coloring agent such as titanium dioxide, a filler such as barium sulfate, a dispersant, an antioxidant, an ultraviolet absorber, a photostabilizer, a fluorescent agent, a fluorescent brightener, and the like. The resin composition may also include a powder of metal with a high specific gravity, such as tungsten and molybdenum, in order to adjust the specific gravity thereof.

The thickness of the intermediate layer 2 is preferably 0.2 mm or more, and particularly preferably 0.3 mm or more. On the other hand, the thickness of the intermediate layer 2 is preferably 2.5 mm or less, and particularly preferably 2.2 mm or less. The specific gravity of the intermediate layer 2 is preferably 0.90 or more, and particularly preferably 0.95 or more. The specific gravity of the intermediate layer 2 is preferably 1.10 or less, and particularly preferably 1.05 or less. The intermediate layer 2 may have two or more layers. For example, it is possible to arrange a reinforcing layer outside the intermediate layer 2.

### 1-3. Cover

The cover 3 is made of a resin composition. Polyurethane is a preferable base polymer for the resin composition. The resin composition may include thermoplastic polyurethane or thermosetting polyurethane. From the viewpoint of productivity, thermoplastic polyurethane is preferable. Thermoplastic polyurethane includes a polyurethane component as a hard segment and a polyester component or a polyether component as a soft segment.

Examples of a hardener for the polyurethane component include alicyclic diisocyanate, aromatic diisocyanate, and aliphatic diisocyanate. Alicyclic diisocyanate is particularly preferable. Since alicyclic diisocyanate has no double bonds in its main chain, the yellowing of the cover 3 is suppressed. Examples of alicyclic diisocyanate include 4,4'-dicyclohexylmethane diisocyanate (H12MDI), 1,3-bis(isocyanatomethyl)cyclohexane (H6XDI), isophorone diisocyanate (IPDI), and trans-1,4-cyclohexane diisocyanate (CHDI). From the viewpoint of versatility and processability, H12MDI is preferable.

The resin composition of the cover 3 may include another polymer instead of polyurethane. Other examples of polymers include an ionomer resin, polystyrene, polyamide, polyester, and polyolefin. The resin composition may include two or more types of polymers.

The resin composition of the cover 3 may include a coloring agent such as titanium dioxide, a filler such as barium sulfate, a dispersant, an antioxidant, an ultraviolet absorber, a photostabilizer, a fluorescent agent, a fluorescent brightener, and the like.

The thickness of the cover 3 is preferably 0.2 mm or more, and particularly preferably 0.3 mm or more. The thickness of the cover 3 is preferably 2.5 mm or less, and particularly preferably 2.2 mm or less. The specific gravity of the cover 3 is preferably 0.90 or more, and particularly preferably 0.95 or more. The specific gravity of the cover 3 is preferably 1.10 or less, and particularly preferably 1.05 or less. It should be noted that the cover 3 may have two or more layers.

Dimples 5 are formed on the surface of the cover 3. In FIG. 2, a virtual line T indicates a common tangent of two ends of the dimple 5. The volume of a portion enclosed by the virtual line T and the surface of the dimple 5 is the volume of the dimple 5. The total volume of the dimples 5 is preferably 270 mm³ or more and 370 mm³ or less. If the total volume is less than the above-described range, the trajectory of the golf ball sometimes rises. From this viewpoint, the total volume is more preferably 290 mm³ or more. If the total volume is more than the above-described range, there is a risk that the trajectory of the golf ball drops. From this viewpoint, the total volume is more preferably 350 mm³ or less.

The ratio of the total area of the dimples 5 to the surface area of a virtual sphere is referred to as "surface area occupation ratio". The surface area occupation ratio is preferably 70% or more and 90% or less. If the surface area occupation ratio is less than the above-described range, there is a risk that lift of the golf ball during flight becomes insufficient. From this viewpoint, the surface area occupation ratio is more preferably 72% or more, and particularly preferably 75% or more. On the other hand, if the surface area occupation ratio is more than the above-described range, the trajectory of the golf ball sometimes rises. From this viewpoint, the surface area occupation ratio is preferably 88% or less, and more preferably 86% or less. It should be noted that the area of the dimple 5 is the area of a region surrounded by an edge line (that is, the area of a planar shape) when the center of the golf ball is viewed from infinity.

The depth of each dimple 5 is preferably 0.1 mm or more and 0.6 mm or less. If the depth is less than the above-described range, the trajectory of the golf ball sometimes rises. From this viewpoint, the depth is more preferably 0.12 mm or more, and particularly preferably 0.14 mm or more. On the other hand, if the depth is more than the above-described range, the trajectory of the golf ball sometimes drops. From this viewpoint, the depth is more preferably 0.55 mm or less, and particularly preferably 0.50 mm or less. The ratio of the number of the dimples 5 whose depth is included in the above-described range to the total number of the dimples 5 is preferably 50% or more, more preferably 65% or more, and particularly preferably 80% or more. The depth is the distance from the virtual line T to the deepest portion of the dimple 5.

The total number of the dimples 5 is preferably 200 or more and 500 or less. If the total number is less than the above-described range, it is difficult to obtain the effects of the dimples. From this viewpoint, the total number is more preferably 230 or more, and particularly preferably 260 or more. On the other hand, if the total number is more than the above-described range, it is difficult to obtain the effects of the dimples. From this viewpoint, the total number is more preferably 470 or less, and particularly preferably 440 or less.

It should be noted that a single type of or a plurality of types of the dimples 5 may be formed. Noncircular dimples (dimples whose planar shape is noncircular) may be formed instead of or together with the circular dimples 5.

### 1-4. Coating layer

Next, the coating layer 4 will be described. The coating layer 4 is configured by covering the surface of the cover 3 with paint. For example, a clear paint containing two-part curable polyurethane as a base material can be used as such paint, but there is no particular limitation as long as paint is used.

The thickness of the coating layer 4 is preferably 5.0 µm or more, more preferably 5.5 µm or more, and particularly preferably 6.0 µm or more. This is because if the thickness of the coating layer 4 is less than 5.0 µm, there is a risk that the coating layer 4 comes off the cover 3 in a step of forming roughness, which will be described later. On the other hand, there is no particular limitation on the upper limit of the thickness of the coating layer 4, but if the thickness of the coating layer 4 is increased by increasing the amount of paint applied, for example, there is a high possibility that the thickness of the coating layer 4 of the entire ball does not become uniform. From this viewpoint, the thickness of the coating layer 4 is preferably 30 µm or less.

Furthermore, roughness is formed on the surface of the coating layer 4. That is, as described later, after the smooth coating layer 4 is formed on the cover 3, roughness is formed on the surface of the coating layer 4. The roughness is for enhancing the aerodynamic effect of the golf ball, and is formed in view of the following.

Here, forces shown in FIG. 3 act on a golf ball that has been hit. That is, gravity, drag due to air in the direction opposite to the flight direction, and lift due to spin of the ball act on the ball. Accordingly, a vector F of the force acting on the ball is expressed by the following expression. $F = {F}_{L} + {F}_{D} + {F}_{G}$
F_{L} : Lift vector
F_{D} : Drag vector
F_{G} : Gravity vector

The lift vector and the drag vector are respectively expressed by the following expressions. ${F}_{L} = 0.5 * CL * ρ * A * {V}^{2}$ ${F}_{D} = 0.5 * CD * ρ * A * {V}^{2}$
CD: Drag coefficient
CL: Lift coefficient
p: Air density
A: Projected area of golf ball
V: Velocity of golf ball

It should be noted that the drag coefficient CD and the lift coefficient CL are measured in an ITR (Indoor Test Range) prescribed in the rules of the USGA.

Accordingly, in order to extend the flight-distance, it is necessary to reduce both the CD and the CL. Therefore, in the golf ball according to this embodiment, as the condition 1, roughness is formed on the surface of the coating layer 4 such that the relationship between a drag coefficient CD1 and a lift coefficient CL1 when the golf ball is hit under the condition in which the Reynolds number is 1. 771×10⁵ and the spin amount is 2280 rpm satisfies CD1×CL1<0.0370 (Expression 4).

In addition to forming roughness so as to satisfy the relationship between the aerodynamic characteristics under the condition 1, it is also possible to form roughness so as to satisfy the relationship between the aerodynamic characteristics under the following condition 2. That is, as the condition 2, it is also possible to form roughness on the surface of the coating layer 4 such that the relationship between a drag coefficient CD2 and a lift coefficient CL2 when the golf ball is hit under the condition in which the Reynolds number is 1.771×10⁵ and the spin amount is 2940 rpm satisfies CD2xCL2<0.0410 (Expression 5).

Both the conditions 1 and 2 are close to the initial condition when a golf ball is hit by a somewhat hard-hitter among average golfers. More specifically, in the condition 1, a spin amount that is close to the spin amount given to a golf ball on average is assumed, and in the condition 2, a spin amount that is more than the spin amount given to a golf ball on average is assumed. The inventors of the present invention found that if the relationships that the drag coefficients CD1 and CD2 have with the lift coefficients CL1 and CL2 are satisfied as described above in the above conditions 1 and 2, the flight-distance is increased. For example, if the condition 1 is satisfied, an increase in the flight-distance can be expected for average golfers. Furthermore, if the condition 2 is satisfied, the above-described effect can be expected to be obtained even in the case of golfers for which the ball rises too high due to a large amount of spin or average golfers who give too much spin to the ball due to a mishit. With a golf ball that satisfies both of the conditions 1 and 2, it is possible to obtain the effect of extending the flight-distance under most spin conditions of average golfers, particularly in the case of giving a large amount of spin.

In order to obtain the aerodynamic characteristics as described above, it is possible to form roughness by various methods. For example, it is possible to obtain the above-described aerodynamic characteristics by setting a maximum height Rz and an arithmetic average roughness Ra of the surface of the coating layer 4 as follows.

That is, the arithmetic average roughness Ra of the coating layer 4 is preferably 0.5 µm or more, more preferably 0.6 µm or more, and particularly preferably 0. 7 µm or more. This is because if the arithmetic average roughness Ra is less than 0.5 µm, a sufficient aerodynamic effect due to roughness cannot be obtained. On the other hand, there is no particular limitation on the upper limit of the arithmetic average roughness Ra, but if roughness is increased, there is a possibility that intimate contact failure of the coating layer 4 with the cover 3 occurs or the coating layer 4 comes off the cover 3, and therefore the arithmetic average roughness Ra is preferably 5 µm or less.

On the other hand, the maximum height Rz is preferably 4.0 µm or more, more preferably 4.5 µm or more, and particularly preferably 5.0 µm or more. This is because if the maximum height Rz is less than 4.0 um, a sufficient aerodynamic effect due to roughness cannot be obtained. On the other hand, there is no particular limitation on the upper limit of the maximum height Rz, but if roughness is increased, there is a possibility that intimate contact failure of the coating layer 4 with the cover 3 occurs or the coating layer 4 comes off the cover 3, and therefore the maximum height Rz is preferably 20 µm, or less. It should be noted that the maximum height Rz and the arithmetic average roughness Ra are measured in accordance with JIS B0601 (2001).

### 2. Method for producing golf ball

The golf ball is produced as follows. Known methods are used as a method for producing such a golf ball as appropriate. First, the core 1 is molded, and the intermediate layer 2 and the cover 3 are molded around the core 1 in this order. The dimples 5 are formed simultaneously with the molding of the cover 3. That is, a cavity of a metal mold for molding the cover is provided with a large number of raised portions for molding the dimples. Next, paint is applied to the surface of the cover 3. The coating layer 4 can be obtained by drying this paint.

There is no particular limitation on the painting method when using curable paint, and known methods can be used. Examples thereof include spray painting and electrostatic painting.

When spray painting using an air gun is performed, a mixture obtained by supplying a polyol component and a polyisocyanate component using respective pumps and by continuously mixing them using a line mixer disposed just in front of the air gun may be applied by spraying, or polyol and polyisocyanate may be separately applied by spraying using an air spray system including a mixing ratio control mechanism. Coating may be achieved at one time by a spray application or may be repeated multiple times.

The curable paint that has been applied to the golf ball body can form a coating by being dried at a temperature of 30 to 70°C for 1 to 24 hours, for example.

### 3. Method for forming roughness of coating layer

Next, a method for forming roughness of the coating layer 4 will be described. There are various methods for forming roughness of the coating layer 4, such as the following two methods.

### 3-1. Surface treatment by spraying minute particles

In this method, roughness is formed by spraying minute particles onto the surface of the coating layer 4. It is possible to spray minute particles with an air gun or the like onto the entire surface while rotating the ball, for example. It is desirable that the spraying pressure at this time is 1 to 10 bar. This is because a spraying pressure that is less than 1 bar makes it difficult to obtain the desired roughness, whereas a spraying pressure that is more than 10 bar causes a risk that not only the coating layer 4 but also the cover 3 are damaged.

Various types of minute particles can be used as the minute particles used in this method. Examples thereof include a natural ore, synthetic resin, and ceramic-based particles. For example, SiC, SiO₂, AL₂O₃, MgO, and Na₂O, or a mixture thereof can be used as a natural ore, and a thermoplastic resin and thermosetting resin that contain melamine-based resin as a main component, or a mixture thereof can be used as a synthetic resin. Moreover, one example of the ceramic-based particles is metal oxide such as zirconia. However, it is preferable to use minute particles having an average particle diameter of 50 µm or more in order to obtain the desired roughness. There is no particular limitation on the upper limit of the average particle diameter of minute particles, but if the particle diameter is increased, there is a possibility that it becomes difficult to spray the particles, and therefore, the average particle diameter is preferably 500 µm or less.

It should be noted that if the thickness of the coating layer 4 is too small when roughness is formed by this method, there is a risk that the coating layer 4 comes off during the spraying of minute particles. From this viewpoint, the thickness of the coating layer 4 is as described above.

### 3-2. Pressing treatment

In this method, the desired roughness is formed by performing pressing treatment using a metal mold in which roughness has been formed on the inner wall surface of the cavity after the coating layer 4 is formed. Accordingly, the desired roughness is formed on the inner wall surface of the cavity in advance. There is no particular limitation on the metal mold used in this method as long as roughness is formed, and, for example, the same metal mold used to mold the dimples can be used. Roughness can be formed in advance on the inner wall surface of the cavity by spraying minute particles as described above.

It should be noted that if the thickness of the coating layer 4 is too small when roughness is formed by this method, it is difficult to form the desired roughness. From this viewpoint, the thickness of the coating layer 4 is as described above.

Although an embodiment of the present invention has been described above, the present invention is not limited to the above embodiment, and various modifications can be carried out without departing from the spirit of the invention. For example, as described above, there is no particular limitation on the number of layers of the core 1, the intermediate layer 2, and the cover 3, and it is sufficient to cover at least the surface of the member at the outermost layer with the coating layer. It should be noted that the above-described embodiment is configured by three layers that are the core 1, the intermediate layer 2, and the cover 3, and the intermediate layer and the cover correspond to a cover member of the present invention. Moreover, a two-piece structure including the core and the cover can be also achieved.

### Examples

Hereinafter, examples of the present invention will be described. However, the present invention is not limited to the following examples.

Here, eight types of golf balls in total including Working Examples 1 to 6 and Comparative Examples 1 and 2 were examined. These golf balls have the same basic specifications, but differ from each other in surface roughness, CD, and CL. Accordingly, first, the common specifications will be described.

### Common specifications

A rubber composition was obtained by kneading 100 parts by mass of high-cis polybutadiene (product name "BR-730" manufactured by JSR Corporation), 35 parts by mass of zinc acrylate, 5 parts by mass of zinc oxide, 5 parts by mass of barium sulfate, 0.5 parts by mass of diphenyl disulfide, 0.9 parts by mass of dicumyl peroxide and 2.0 parts by mass of zinc octanoate. This rubber composition was placed into a metal mold configured by an upper mold and a lower mold, both of which have a semispherical cavity, and was heated at 170°C for 18 minutes, and thus a core having a diameter of 39.7 mm was obtained.

A resin composition was obtained by kneading 50 parts by mass of an ionomer resin (product name "Surlyn 8945" manufactured by Du Pont), 50 parts by mass of another ionomer resin (product name "Himilan AM7329" manufactured by Du Pont-Mitsui Polychemicals), 4 parts by mass of titanium dioxide, and 0.04 parts by mass of ultramarine blue using a twin-screw kneading extruder. An intermediate layer was formed by covering the core with this resin composition by an injection molding method. The thickness of this intermediate layer was 1.0 mm.

A paint composition (product name "Polin 750LE" manufactured by Shinto Paint Co., Ltd.) containing a two-part curable epoxy resin as a base polymer was prepared. The main agent liquid for the paint composition is constituted by 30 parts by mass of a bisphenol A-type solid epoxy resin and 70 parts by mass of a solvent. The curing agent liquid for the paint composition is constituted by 40 parts by mass of modified polyamide amine, 55 parts by mass of a solvent, and 5 parts by mass of titanium oxide. The mass ratio of the main agent liquid and the curing agent liquid is 1/1. The paint composition was applied to the surface of the intermediate layer using a spray gun, and was allowed to stand under the atmosphere at 23°C for 6 hours, and thus a reinforcing layer was obtained. The thickness of this reinforcing layer was 10 µm.

A resin composition was obtained by kneading 100 parts by mass of a thermoplastic polyurethane elastomer (product name "Elastollan XNY85A" manufactured by BASF Japan Ltd.) and 4 parts by mass of titanium dioxide using a twin-screw extruder. Half shells were made of this resin composition by a compression molding method. A sphere configured by the core, the intermediate layer, and the reinforcing layer was covered with the two half shells. The half shells and the sphere were placed into a final metal mold configured by an upper mold and a lower mold, both of which have a semispherical cavity and have a large number of pimples on the surface of the cavity, and then a cover was formed by a compression molding method. The thickness of the cover was 0 . 5 mm. The cover was provided with dimples having an inverted shape of the pimple. A coating layer was formed by applying a clear paint containing two-part curable polyurethane as a base material around the cover.

Specifically, the golf ball body was mounted on a rotator, and then the clear paint was applied while rotating the rotator at 300 rpm and vertically moving an air gun that was separated from the golf ball body by a spraying distance (7 cm). Each interval between the repeated applications was set to 1.0 second. The paint was applied using an air gun under the spraying condition in which the spraying air pressure was 0.15 MPa, the force feeding tank air pressure was 0.10 MPa, the single application time was 1 second, the atmospheric temperature was 20 to 27°C, and the atmospheric humidity was 65% or less.

In all of the working examples and comparative examples, the thickness of the coating layer was 18 µm, and clear paint was applied twice. As a result, golf balls having a diameter of about 42.7 mm and a mass of about 45.6 g were obtained. The compressive deformation amount measured by a YAMADA compression tester when setting the load to 98 to 1274 N was about 2.45 mm. Table 1 shows the specifications of the dimples of the golf ball.

**Table 1**

| Type | Number | Diameter Dm (mm) | Depth Dp (mm) | Curvature CR (mm) | Spherical surface area s (mm²) | Volume (mm³) |
|---|---|---|---|---|---|---|
| A | 16 | 4.600 | 0.259 | 19.66 | 16.67 | 2.157 |
| B | 30 | 4.500 | 0.254 | 18.82 | 15.95 | 2.021 |
| C | 30 | 4.400 | 0.249 | 17.99 | 15.25 | 1.892 |
| D | 150 | 4.300 | 0.244 | 17.19 | 14.56 | 1.770 |
| E | 30 | 4.200 | 0.239 | 16.40 | 13.89 | 1.654 |
| F | 66 | 4.100 | 0.234 | 15.63 | 13.23 | 1.544 |
| G | 10 | 3.800 | 0.220 | 13.44 | 11.36 | 1.247 |
| H | 12 | 3.400 | 0.203 | 10.77 | 9.09 | 0.922 |

### Working Examples

In Working Examples 1 to 6, roughness was formed on the surface of the coating layer of the golf ball obtained as described above by the following method. That is, after the coating layer was formed, minute particles were sprayed thereon using an air gun having a nozzle diameter of 8 mm. At this time, 20 balls of each working example were placed into a predetermined treatment device, and minute particles were sprayed thereon with a predetermined pressure for 1 minute while rotating the device. The pressure at this time and minute particles used are as shown in Table 2.

### Comparative Examples

In Comparative Example 1, after the coating layer was formed, surface treatment was not performed on its surface. In Comparative Example 2, as in the above-described working examples, after the coating layer was formed, roughness was formed by spraying minute particles. The pressure at this time and minute particles used are as shown in Table 2.

The maximum height Rz, the arithmetic average roughness Ra, the above-described CD1, CD2, CL1, CL2,and the like in the working examples and comparative examples, which were formed as described above, are as shown in Table 2.

**Table 2**

| | Work. Ex. 1 | Work. Ex. 2 | Work. Ex. 3 | Work. Ex. 4 | Work. Ex. 5 | Work. Ex. 6 | Comp. Ex. 1 | Comp. Ex. 2 |
|---|---|---|---|---|---|---|---|---|
| Type | Synthetic resin | Ceramic-based particle | Natural ore | Natural ore | Natural ore | Natural ore | | Natural ore |
| Particle diameter (um) | 75-150 | 75-150 | 75-150 | 75-150 | 75-150 | 250-500 | | 30-50 |
| Pressure (bar) | 1.5 | 1.5 | 3.5 | 5.5 | 7.5 | 5.5 | | 1.5 |
| Ra (µm) | 0.57 | 0.75 | 0.77 | 0.93 | 1.04 | 1.51 | 0.36 | 0.48 |
| Rz (µm) | 4.92 | 5.4 | 6.52 | 6.9 | 7.7 | 10.1 | 1.12 | 2.5 |
| CD1 | 0.229 | 0.229 | 0.228 | 0.228 | 0.227 | 0.226 | 0.23 | 0.23 |
| CL1 | 0.161 | 0.16 | 0.16 | 0.159 | 0.158 | 0.157 | 0.162 | 0.161 |
| CD2 | 0.232 | 0.231 | 0.23 | 0.229 | 0.228 | 0.227 | 0.233 | 0.232 |
| CL2 | 0.178 | 0.178 | 0.176 | 0.175 | 0.175 | 0.174 | 0.18 | 0.179 |
| CD1×CL1 | 0.0369 | 0.0366 | 0.0365 | 0.0363 | 0.0359 | 0.0355 | 0.0373 | 0.037 |
| CD2×CL2 | 0.0413 | 0.0411 | 0.0405 | 0.0401 | 0.0399 | 0.0395 | 0.0419 | 0.0415 |

The maximum height Rz and the arithmetic average roughness Ra were measured using a surface roughness measuring instrument (Surfcom 130A manufactured by Tokyo Seimitsu Co., Ltd.). Six balls of each of the working examples and comparative examples were prepared, roughness was measured at six points in a dimple of each ball, and the average values were used as the Rz and the Ra.

### Evaluation test

A flight-distance test was performed on the working examples and comparative examples formed as described above.

### Flight-distance test

A metal head driver (product name "SRIXON Z525" (W#1) manufactured by Dunlop Sports Co. , Ltd. ; carbon shaft hardness: S, loft angle: 9.5°) was attached to a swing machine manufactured by Golf Laboratories Inc. The head speed was set to 47 m/s, and the swing machine was adjusted such that the ball speed was 67 m/sec, the launch angle was 12.5°, and the spin amount was 2600 rpm when using the balls of Comparative Example 1. Then, 20 balls of each of the working examples and comparative examples were hit, the distance (total) to the point where the ball stopped was measured, and the average was examined. It should be noted that when the test was performed, substantially no wind blew. Table 3 shows the results.

**Table 3**

| | Work. Ex. 1 | Work. Ex. 2 | Work. Ex. 3 | Work. Ex. 4 | Work. Ex. 5 | Work. Ex. 6 | Comp. Ex. 1 | Comp. Ex. 2 |
|---|---|---|---|---|---|---|---|---|
| Total (m) | 240.7 | 240.9 | 241.2 | 241.4 | 241.8 | 241.5 | 240 | 240.2 |
| Trajectory height (m) | 26 | 25.9 | 25.8 | 25.7 | 25.6 | 25.3 | 26.5 | 26.4 |

### Evaluation

As shown in Tables 2 and 3, in the flight-distance test, the trajectories of the working examples were generally lower than those of the comparative examples. That is, it is thought that lift and drag were reduced due to setting roughness of the coating films of the working examples so as to satisfy Expression 4. As a result, the flight-distances of all of the working examples were extended compared with those of the comparative examples. Moreover, in Working Examples 3 to 6, which also satisfied Expression 5, the trajectory height was lowered compared with those of Working Examples 1 and 2, which satisfied only Expression 4, and the flight-distance was further extended.

## Claims

1. A golf ball comprising:
a spherical core (1);
at least one cover member (3) that covers the core (1); and
a coating layer (4) that covers the cover member (3) configuring an outermost layer,
wherein a plurality of dimples are formed in the cover member (3) configuring the outermost layer, **characterized in that**
roughness is formed on a surface of the coating layer (4) such that a relationship between a drag coefficient CD1 and a lift coefficient CL1 when a golf ball is hit with a Reynolds number of 1.771×10⁵ and a spin amount of 2280 rpm satisfies CD1×CL1<0.0370.

2. The golf ball according to claim 1, wherein roughness is formed on the surface of the coating layer (4) such that a relationship between a drag coefficient CD2 and a lift coefficient CL2 when a golf ball is hit with a Reynolds number of 1.771×10⁵ and a spin amount of 2940 rpm satisfies CD2×CL2<0.0410.

3. The golf ball according to claim 1 or 2, wherein an arithmetic average roughness Ra of the surface of the coating layer (4) is 0.5 µm or more.

4. The golf ball according to claim 1 or 2, wherein a maximum height Rz is 4.0 µm or more.

5. The golf ball according to claim 1 or 2, wherein an arithmetic average roughness Ra of the surface of the coating layer (4) is 0.5 µm or more and a maximum height Rz is 4.0 µm or more.

6. The golf ball according to any one of claims 1 to 5, wherein the roughness of the coating layer (4) is formed by spraying minute particles.

7. The golf ball according to claim 6, wherein an average particle diameter of the minute particles is 50 µm or more.

8. The golf ball according to any one of claims 1 to 7, wherein the thickness of the coating layer (4) is 5.0 µm or more and 30 µm or less.

9. A method for producing a golf ball comprising:
a step of forming a spherical core (1);
a step of covering the spherical core (1) with at least one cover member (3) and forming a plurality of dimples in the cover member (3) configuring an outermost layer;
a step of covering the cover member (3) configuring the outermost layer with a coating layer (4); **characterized in that** the method further comprises:
a step of forming roughness on a surface of the coating layer (4) such that a relationship between a drag coefficient CD1 and a lift coefficient CL1 when a golf ball is hit with a Reynolds number of 1.771×10⁵ and a spin amount of 2280 rpm satisfies CD1×CL1<0.0370.

10. The method for producing a golf ball according to claim 9, wherein in the step of forming roughness, roughness is formed on the surface of the coating layer (4) such that a relationship between a drag coefficient CD2 and a lift coefficient CL2 when a golf ball is hit with a Reynolds number of 1.771×10⁵ and a spin amount of 2940 rpm satisfies CD2×CL2<0.0410.

11. The method for producing a golf ball according to claim 9 or 10, wherein an arithmetic average roughness Ra of the surface of the coating layer (4) is 0.5 µm or more.

12. The method for producing a golf ball according to claim 9 or 10, wherein a maximum height Rz is 4.0 µm or more.

13. The method for producing a golf ball according to claim 9 or 10, wherein an arithmetic average roughness Ra of the roughness formed on the surface of the coating layer (4) is 0.5 µm or more and a maximum height Rz is 4.0 µm or more.

14. The method for producing a golf ball according to any one of claims 9 to 13, wherein the roughness of the coating layer is formed by spraying minute particles.

15. The method for producing a golf ball according to claim 13, wherein an average particle diameter of the minute particles is 50 µm or more.

## Patentansprüche

1. Golfball, umfassend:
einen kugelförmigen Kern (1);
zumindest ein Abdeckelement (3), das den Kern (1) bedeckt; und
eine Beschichtungslage (4), die das Abdeckelement (3) bedeckt und eine äußerste Lage ausbildet,
wobei eine Mehrzahl von Dimples in dem Abdeckelement (3), das die äußerste Lage ausbildet, gebildet ist, **dadurch gekennzeichnet, dass**
eine Rauheit auf einer Oberfläche der Beschichtungslage (4) gebildet ist, so dass eine Beziehung zwischen einem Widerstandsbeiwert CD1 und einem Auftriebsbeiwert CL1, wenn der Golfball mit einer Reynolds-Zahl von 1,771×10⁵ und einem Spinbetrag von 2280 U/min geschlagen wird, CD1×CL1 <0,0370 erfüllt.

2. Golfball nach Anspruch 1, wobei die Rauheit auf der Oberfläche der Beschichtungslage (4) derart gebildet ist, dass eine Beziehung zwischen einem Widerstandsbeiwert CD2 und einem Auftriebsbeiwert CL2, wenn ein Golfball mit einer Reynolds-Zahl von 1,771×10⁵ und einem Spinbetrag von 2940 U/min geschlagen wird, CD2xCL2<0,0410 erfüllt.

3. Golfball nach Anspruch 1 oder 2, wobei die arithmetische Mittenrauheit Ra der Oberfläche der Beschichtungslage (4) 0,5 µm oder mehr beträgt.

4. Golfball nach Anspruch 1 oder 2, wobei die maximale Rautiefe Rz 4,0 µm oder mehr beträgt.

5. Golfball nach Anspruch 1 oder 2, wobei die arithmetische Mittenrauheit Ra der Oberfläche der Beschichtungslage (4) 0,5 µm oder mehr beträgt und die maximale Rautiefe Rz 4,0 µm oder mehr beträgt.

6. Golfball nach einem der Ansprüche 1 bis 5, wobei die Rauheit der Beschichtungslage (4) durch Aufsprühen winziger Partikel gebildet ist.

7. Golfball nach Anspruch 6, wobei der durchschnittliche Partikeldurchmesser der winzigen Partikel 50 µm oder mehr beträgt.

8. Golfball nach einem der Ansprüche 1 bis 7, wobei die Dicke der Beschichtungslage (4) 5,0 µm oder mehr und 30 µm oder weniger beträgt.

9. Verfahren zum Herstellen eines Golfballs, umfassend:
einen Schritt eines Bildens eines kugelförmigen Kerns (1);
einen Schritt eines Bedeckens des kugelförmigen Kerns (1) mit zumindest einem Abdeckelement (3) und Bilden einer Mehrzahl von Dimples in dem Abdeckelement (3), das als äußerste Lage ausgebildet worden ist;
einen Schritt eines Bedeckens des Abdeckelements (3), das die äu-ßerste Lage ausbildet, mit einer Beschichtungslage (4); **dadurch gekennzeichnet, dass** das Verfahren ferner umfasst:
einen Schritt eines Bildens einer Rauheit auf einer Oberfläche der Beschichtungslage (4), so dass eine Beziehung zwischen einem Widerstandsbeiwert CD1 und einem Auftriebsbeiwert CL1, wenn der Golfball mit einer Reynolds-Zahl von 1,771×10⁵ und einem Spinbetrag von 2280 U/min geschlagen wird, CD1×CL1<0,0370 erfüllt.

10. Verfahren zum Herstellen eines Golfballs nach Anspruch 9, wobei bei dem Schritt eines Bildens einer Rauheit die Rauheit auf der Oberfläche der Beschichtungslage (4) derart gebildet wird, dass eine Beziehung zwischen einem Widerstandsbeiwert CD2 und einem Auftriebsbeiwert CL2, wenn ein Golfball mit einer Reynolds-Zahl von 1,771×10⁵ und einem Spinbetrag von 2940 U/min geschlagen wird, CD2xCL2<0,0410 erfüllt.

11. Verfahren zum Herstellen eines Golfballs nach Anspruch 9 oder 10, wobei die arithmetische Mittenrauheit Ra der Oberfläche der Beschichtungslage (4) 0,5 µm oder mehr beträgt.

12. Verfahren zum Herstellen eines Golfballs nach Anspruch 9 oder 10, wobei die maximale Rautiefe Rz 4,0 µm oder mehr beträgt.

13. Verfahren zum Herstellen eines Golfballs nach Anspruch 9 oder 10, wobei die arithmetische Mittenrauheit Ra der Rauheit, die auf der Oberfläche der Beschichtungslage (4) gebildet wird, 0,5 µm oder mehr beträgt, und die maximale Rautiefe Rz 4,0 µm oder mehr beträgt.

14. Verfahren zum Herstellen eines Golfballs nach einem der Ansprüche 9 bis 13, wobei die Rauheit der Beschichtungslage durch Aufsprühen von winzigen Partikeln gebildet wird.

15. Verfahren zum Herstellen eines Golfballs nach Anspruch 13, wobei der durchschnittliche Partikeldurchmesser der winzigen Partikel 50 µm oder mehr beträgt.

## Revendications

1. Balle de golf comprenant :
un noyau sphérique (1) ;
au moins un élément de couverture (3) qui couvre le noyau (1) ; et
une couche de revêtement (4) qui couvre l'élément de couverture (3), configurant une couche tout à fait extérieure,
dans laquelle une pluralité de petites cuvettes sont formées dans l'élément de couverture (3) configurant la couche tout à fait extérieure,
**caractérisé en ce que**
une rugosité est formée sur une surface de la couche de revêtement (4) de telle façon qu'une relation entre un coefficient de traînée (CD1) et un coefficient de portance (CL1) quand une balle de golf est frappée avec un nombre de Reynolds de 1,771 x 10⁵, et une vitesse de rotation de 2280 tr/m satisfait la relation suivante CD1 x CL1 < 0,0370.

2. Balle de golf selon la revendication 1, dans laquelle la rugosité est formée sur la surface de la couche de revêtement (4) de telle façon qu'une relation entre un coefficient de traînée CD2 et un coefficient de portance CL2 quand une balle de golf est frappée avec un nombre de Reynolds de 1,771 x 10⁵ et une vitesse de rotation de 2940 tr/mn satisfait la relation suivante CD2 x CL2 < 0,0410.

3. Balle de golf selon la revendication 1 ou 2, dans laquelle une rugosité moyenne arithmétique Ra de la surface de la couche de revêtement (4) est de 0,5 µm ou plus.

4. Balle de golf selon la revendication 1 ou 2, dans laquelle une hauteur maximum Rz est de 4,0 µm ou plus.

5. De golf selon la revendication 1 ou 2, dans laquelle une rugosité moyenne arithmétique Ra de la surface de la couche de revêtement (4) est de 0,5 µm ou plus et une hauteur maximum Rz est de 4,0 µm ou plus.

6. Balle de golf selon l'une quelconque des revendications 1 à 5, dans laquelle la rugosité de la couche de revêtement (4) est formée en pulvérisant des particules minuscules.

7. Balle de golf selon la revendication 6, dans laquelle un diamètre de particules moyen des particules minuscules et de 50 µm ou plus.

8. Balle de golf selon l'une quelconque des revendications 1 à 7, dans laquelle l'épaisseur de la couche de revêtement (4) et de 5,0 µm ou plus et 30 µm ou moins.

9. Procédé pour produire une balle de golf, comprenant :
une étape pour former un noyau sphérique (1) ;
une étape pour couvrir le noyau sphérique (1) avec au moins un élément de couverture (3) et pour former une pluralité de petites cuvettes dans l'élément de couverture (3) configurant une couche tout à fait extérieure ;
une étape pour couvrir l'élément de couverture (3) configurant la couche tout à fait extérieure, avec une couche de revêtement (4) ;
**caractérisé en ce que** le procédé comprend en outre :
une étape pour former une rugosité sur une surface de la couche de revêtement (4) de telle façon qu'une relation entre un coefficient de traînée CD1 et un coefficient de portance CL1 quand une balle de golf est frappée avec un nombre de Reynolds de 1,771 x 10⁵ et une vitesse de rotation de 2280 tr/mn satisfait la relation CD1 x CL1 < 0,0370.

10. Procédé pour produire une balle de golf selon la revendication 1, dans lequel, dans l'étape pour former une rugosité, la rugosité est formée sur la surface de la couche de revêtement (4) de telle façon qu'une relation entre un coefficient de traînée CD2 et un coefficient de portance CL2 quand une balle de golf est frappée avec un nombre de Reynolds de 1,771 x 10⁵ et une vitesse de rotation de 2940 tr/mn satisfait la relation CD2 x CL2 < 0,0410.

11. Procédé pour produire une balle de golf selon la revendication 9 ou 10, dans lequel une rugosité moyenne arithmétique Ra de la surface de la couche de revêtement (4) est de 0,5 µm ou plus.

12. Procédé pour produire une balle de golf selon la revendication 9 ou 10, dans lequel une hauteur maximum Rz est de 4,0 µm ou plus.

13. Procédé pour produire une balle de golf selon la revendication 9 ou 10, dans lequel une rugosité moyenne arithmétique Ra de la rugosité formée sur la surface de la couche de revêtement (4) est de 0,5 µm ou plus et une hauteur maximum Rz est de 4,0 µm ou plus.

14. Procédé pour produire une balle de golf selon l'une quelconque des revendications 9 à 13, dans lequel la rugosité de la couche de revêtement est formée en pulvérisant des particules minuscules.

15. Procédé pour produire une balle de golf selon la revendication 13, dans lequel un diamètre de particules moyen des particules minuscules est de 50 µm ou plus.
